

Dec. 17, 1935.

H. G. McILVRIED

2,025,002

METHOD OF ROLLING SHEET METALS

Filed Dec. 29, 1933

3 Sheets-Sheet 1



Fig. 1.

*Inventor:*  
HOWARD G. McILVRIED,  
*by:* *Usina & Rubber*  
*his Attorneys.*

Dec. 17, 1935.

H. G. McILVRIED

2,025,002

## METHOD OF ROLLING SHEET METALS

Filed Dec. 29, 1933

3 Sheets-Sheet 2



*Inventor:*

HOWARD G. MCILVRIED,

by: Usina & Rauber  
his Attorneys.

Dec. 17, 1935.

H. G. McILVRIED

2,025,002

METHOD OF ROLLING SHEET METALS

Filed Dec. 29, 1933

3 Sheets-Sheet 3



Inventor:  
HOWARD G. McILVRIED,  
by: *Usina & Rauber*  
his Attorneys.

## UNITED STATES PATENT OFFICE

2,025,002

## METHOD OF ROLLING SHEET METALS

Howard G. McIlvried, Bellevue, Pa., assignor to  
 American Sheet and Tin Plate Company, a corporation of New Jersey

Application December 29, 1933, Serial No. 704,564

6 Claims. (Cl. 29—18)

This invention relates to a method of cold rolling thin, wide strip metal and has for its object the provision of a novel method of cold rolling in which the number of passes necessary to get a desired reduction and commercially flat and uniform gage material is reduced to a minimum.

Prior practice has shown that in the commercial cold reduction of wide, hot finished strip such as, for example, .065" hot finished strip cold reduced to .010", it has been the ultimate aim to produce the desired gage of material by cold rolling in as short a time and with as few passes as possible. The first definite step in this direction was to utilize the conventional two high non-reversing cold mill by reducing the diameter of the rolls as much as possible.

By reducing the size of the rolls, the area of metal contact was decreased and more reduction per pass was accomplished without increasing the pressure on the roll necks and in many cases decreasing the driving load on the power unit. However, as the diameter of the rolls decreased they showed a tendency to be deflected at their centers.

Therefore, in reducing these rolls to a smaller diameter it was necessary to utilize supporting or "back up" rolls such as, for example, a four high mill. These back up rolls, located above and below the top and bottom work rolls, respectively, prevent the majority of the vertical deflection of the small work rolls but do not prevent their horizontal or lateral deflection.

Such a cold reduction mill may commercially be of several types. In the production of wide, thin gaged strip in relatively long lengths such a mill might utilize several stands or mills set in line or tandem. Such mills are non-reversing with the working rolls being driven. Should re-rolling be desired it is necessary to convey the material back to the entering side of such mills by crane or similar conveyance.

Rolling on such a tandem mill, with the material being reduced in several stands simultaneously, necessarily involves very delicate and rapid adjustments of screw pressure, roll contour and speed of the various stands.

Any variation in gage, physical characteristics or composition of the material being rolled or an adjustment of any one stand for any other reason usually necessitates immediate adjustments to one or more other stands in order to produce flat material of the correct final gage. Moreover, tension on the strip on each side of the work rolls has proven in practice to be an essential feature of all types of cold reducing mills and any appreci-

able adjustments on one stand necessitates corresponding adjustments on one or more other stands of the tandem arrangement to preserve the proper tension, which adjustments under running conditions are extremely difficult to obtain with the promptness required to preserve the essential constant tensional effect on the material being reduced.

The interruption of one four high unit in such a tandem train naturally results in a shut down of all other units. Furthermore, a breaking of the strip in one roll unit often causes other breaks and surface wrinkling along the strip in other units before they stop rotating, resulting in possible damage to work roll surfaces requiring roll changes. This results in an excessive amount of lost time and consequent loss of production.

In all probability the major disadvantages in such a train of four high mill lies in the limited amount of product that can be produced in comparison to the initial investment cost.

This is due to the fact that only the last or finishing stand can work at its maximum desired speed. The other units in line (although of practically the same construction and cost) must be operated more slowly, their speed being inversely proportional to the gage of the material delivered from their work rolls.

The operating difficulties as heretofore discussed, together with the high initial investment cost for a low output, naturally results in a high cost per ton of metal so cold reduced. Therefore, the next logical and commercial step, in an endeavor to lower production costs per ton, was the four high reversing mill. This single four high reversing unit eliminated many of the operating difficulties inherent in the tandem train, together with the necessity of slow speeds on the initial reduction.

The strip metal to be cold reduced is fed back and forth between the work rolls which, with the exception of my improved mill, are of extremely small diameter when compared with the work rolls of the four high tandem mill just described.

Thus, for illustrative and comparative purposes only, the approximate ratio of back up and work roll diameters of a four high non-reversing mill described above is approximately two or three to one (2 or 3 to 1) respectively. Contrasted with this mill is the usual four high reversing type mill wherein the ratio of back up and work roll diameters is approximately six to one (6 to 1) respectively, the work rolls usually being under 6" diameter. Ratios for both types of four high cold

reduction mills just described apply to the same size of roll width or face.

This four high reversing mill of the prior art as constructed involves working rolls of extremely small diameter in an effort to reduce the power required to make a predetermined gage reduction. These work rolls are of such a small diameter that they are not mechanically capable of being directly driven with a large power unit. This necessitated other means for conveying the strip through the work rolls which in this case are power driven reels adjacent and on either side of this single reversing mill.

These power driven reels alternately act as tension means for pulling the strip between the work rolls. The reels reverse in such a manner as to cause one reel to be the "tension" or pull reel while at the same time the other reel is the "drag" or unwinding reel. When the strip reaches its end on the drag reel, the direction of movement of metal is reversed with the tension reel and the drag reels interchanging in their function. This reversal is repeated until the desired gage of strip is obtained. This tension is definitely limited in that this pulling action approaches the ultimate strength of the material beyond which it will naturally break.

Moreover, even before the pull is great enough to break the strip, an appreciable horizontal deflection occurs at the center of the very small work rolls. This horizontal deflection causes the work rolls to assume a slightly concave shape which usually results in an excessive ruffling or wrinkling of the edges of the metal. These conditions definitely limit the amount of cold reduction for each pass between the work rolls. Such limited reductions have in practice necessitated 10 to 15 passes through such a mill while reducing relatively soft low carbon, wide hot rolled or finished heavy strip from about 16 USS gage (.065") to about 31 USS gage (.0107").

The above mentioned difficulties in cold reduction of metals are overcome in my method of rolling the same relatively wide hot rolled or finished sheet metal to the same extremely thin gage in less passes than heretofore possible on a single four high reversing cold mill which fact constitutes one of the objects of my herein described invention.

Another object of my invention is to utilize in combination with a limited number of passes of strip metal through a four high cold reduction mill, speeds on initial and intermediate passes not heretofore possible.

A still further object is to utilize a single reversing mill unit which by my methods of cold reduction presents minimum investment costs as well as a minimum operating cost and an increased tonnage output of metal in a given period of time.

These and other objects and advantages of my invention will become apparent in the specifications when considered in conjunction with the illustrative embodiment shown in the accompanying drawings wherein:

Figure 1 indicates a plan view of a single stand, reversing cold rolling mill with motors and reels adjacent thereto, while

Figure 2 shows a side elevation through A—A of Figure 1, and

Figure 3 shows an end view of mill through B—B of Figure 1.

In the drawings I have illustrated a conventional four high reversing cold reduction mill with housings 1 in which are positioned reducing

or work rolls 3 and top and bottom back up rolls 2. The mill housings are mounted on a bed plate 4 which in turn is supported on suitable foundation 5.

The work rolls 3 are driven by the main mill motor 6, power for which is transmitted from the motor to the rolls by means of gear reduction units 7, hence to a flexible coupling 8 and then through pinions 9, couplings 10 and spindles 11. The top back up roll and top work roll are vertically adjustable by means of motors 3<sup>a</sup> and screwdown mechanism 3<sup>b</sup>.

Adjacent and on either side of the main mill are reels 15 and 15<sup>a</sup> which alternately wind and unwind the metal "M". These reels are reversing, being driven by variable speed motors 12 through gear reducers 13 and couplings 14. Into the reel mounts 16 and 16<sup>a</sup> are removably mounted reels or drums 15 and 15<sup>a</sup> onto which the metal M is either coiled or uncoiled, depending on the direction of metal movement.

To illustrate more specifically my invention, as well as to compare its operation with prior cold rolling mills, I will utilize, for example, a heavy 16 (USS) gage (.065") hot rolled and pickled strip or sheet metal which will be reduced to approximately 31 (USS) gage (.0107"). This hot rolled and pickled strip is first wound tightly onto a removable reel 15. The removable reel 15 with its tight coiled hot strip is then mounted onto the reel mount 16 and the strip M is then fed into the cold reduction mill by passing over strip guide 17 and guide plates 18, thence between the work rolls 3 and over corresponding strip guides on the other side of the mill and finally wound onto reel 15<sup>a</sup>, this last mentioned reel now acting as a tension reel whereas the first mentioned reel on which the hot rolled strip is now mounted being for the moment the drag reel.

The work rolls 3 for illustrative purposes will be assumed to have a diameter of approximately about 16" in contrast to the diameters of their respective backing up rolls which have a diameter of approximately about 48". These work and back up roll diameters are for a mill roll having a face or length approximately about 42". Thus it will be noted that I prefer to use a ratio of approximately 3 to 1 between the back up and work rolls, respectively, as contrasted with the ratio of 2 or 3 to 1 on tandem non-reversing cold rolling mills and a ratio of 6 to 1 on a reversing single stand cold rolling mill having rolls not driven, both types of which have been previously described.

This 3 to 1 ratio ultimately aids in giving me a more quickly produced product at less production cost by virtue of the fact that the work rolls are driven and of a size to prevent horizontal deflection together with back up rolls of such a large diameter as to allow screw pressures sufficiently great to accomplish heretofore impossible reductions per pass without their excessive vertical deflection.

To further aid in obtaining my maximum reduction of metal in a limited number of passes either one or both of the work rolls preferably carry a slight convexity which for the size of roll to be utilized in this foregoing example might be as much as .0015" to .0025" crown at the center, or an average increase of diameter of about .0045" at center over the diameter of same roll at both ends.

I find that this convexity of either one or both of the work rolls together with other mechanical improvements herein disclosed, aids

active pass conditions which permit in my single stand more or less the equivalent of what is otherwise accomplished by two or more four-high mills arranged in tandem.

5 Thus for example, this slight convexity of work rolls is lost during the active pass, it being taken up by the spring of the rolls. Such a condition permits each active pass to produce a substantially flat sheet yet leaving sufficient material to finish to a given gage without excessive edge ruffle or center buckle. These mechanical conditions will vary with the starting gage and analysis of the material and during rolling operations the shape and temperature of the metal contacting rolls and screw pressures utilized. All of these conditions are coordinated to produce maximum reduction in a minimum number of passes through the mill to secure the required uniform gage.

20 The motor 6 which drives the work rolls 3 while in the process of reducing strip is capable and does develop power which is greater than the combined and utilized power of both of the real motors 12. Thus, for the size of the mill just described, I prefer to use a mill motor which develops approximately 1200 horse-power as contrasted with reel motors which develop approximately 250 horse-power. It will be obvious to one skilled in the art that with larger mills, 25 rolling wider sheets and hence using wider rolls, that the power utilized, as well as the size of work to back up rolls, will increase with the increased width of metal being reduced.

30 After threading or feeding the strip from one reel through the mill and onto the reel on the opposite side, the mill screws will be operated to adjust the working and back-up rolls so that, when the mill rolls are started and synchronized with the speed of the drag and tension reels, a 35 very decided cold reduction of the metal takes place. In the first or initial pass of the metal to be reduced, I am able to obtain gage reductions and speed of metal not heretofore possible on any type of cold rolling mill.

40 Thus, for illustrative purposes, I may in this first pass cold reduce at a linear speed of about 500 feet per minute, relatively soft, low carbon hot finished sheet or strip having a width of approximately 32", from heavy 16 (USS) gage (.065") to approximately about .032" or heavy 45 22 (USS) gage which is a metal reduction of approximately fifty-one percent (51%).

The mill and the reels are then reversed in 50 their direction of rotation, the mill adjusted for further reduction and the partially reduced strip or sheet metal is simultaneously cold reduced and re-wound onto reel 15. This second cold reduction is at a speed and a gage reduction not heretofore possible as an intermediate pass 55 on any type of cold reduction mill.

60 Thus, for further illustrative purposes, I may in this second pass cold reduce, at a linear speed of about 800 feet per minute, the above mentioned strip from heavy 22 (USS) gage (.032") to approximately about 27 (USS) gage (.017") which is a metal reduction of approximately forty-seven percent (47%).

65 Upon the reversal of the mill and reel motors and adjustment of the mill, the sheet metal or strip is again passed through the cold mill in the same direction as on the first pass. This third, and usually the last, cold reduction is at a speed comparable with the finishing speeds 70 obtainable on other cold reduction mill units.

However, I am able to obtain on my mill a gage reduction which has never to my best knowledge and belief been possible at this point on any single stand reversing cold reduction mill and at a speed not known by me to be possible 75 on the finishing pass of a tandem mill.

Thus, for example, I may cold reduce in this third pass at a linear speed of about 800 feet per minute the gage of the metal being cold reduced from 27 (USS) gage (.017") to about 10 31 gage (USS) (.0107") or lower, giving a gage reduction of about 37 percent.

15 While I have shown and illustrated a method of cold reducing to gages which are most desirable such as the reduction of heavy hot strip to tin plate gages further reductions are possible beyond that described by one or more additional passes.

20 Therefore, to one skilled in the art of cold reducing sheet or strip metal it can be seen that 25 by my method I am able to produce in three or four passes, preferably the former, as above described, a total metal reduction possible only by ten to fifteen passes in other single stand reversing cold mills. It is further noted that I 30 am able to produce by my method speeds on initial and intermediate passes greater than the same passes on tandem cold reducing mills. Speed as mentioned herein is the rate of travel 35 of the strip metal through the cold reducing mill expressed in linear feet of travel per minute.

It is also noted that by my extreme reductions per pass together with high speeds on all passes that I am able to produce in a given 35 period of time tonnages of sheet metal not heretofore possible on any other type of cold reducing mill and hence at a production cost not heretofore possible.

40 Thus, for example, I am able to produce as high as 45 tons in one consecutive eight hour turn or shift, of tin plate stock in 31 (USS) gage, approximately 30 inches wide as cold reduced from heavy hot rolled and pickled 16 (USS) gage.

45 While I have shown and described present preferred embodiments it is understood that various changes and modifications may be made within the scope of the invention and of the following claims.

50 I claim:

1. A method of working a thin and relatively wide metal strip which includes moving the same through a single-stand cold-rolling mill at a linear speed of at least 400 feet per minute, reducing the 55 cross-sectional area of the metal strip at least 35 per cent on its first pass therethrough, and further reducing its cross-sectional area at least an additional 35 per cent while confining the same to not more than three passes after the first pass. 60

2. A method of working a thin and relatively wide metal strip which includes moving the same through a single-stand cold-rolling mill at a linear speed of at least 400 feet per minute, reducing the cross-sectional area of the metal strip 65 approximately 50 per cent on its first pass therethrough, and further reducing its cross-sectional area at least an additional 35 per cent while confining the same to not more than three passes after the first pass. 70

3. A method of working a thin and relatively wide metal strip which includes moving the same through a single-stand cold-rolling mill at a linear speed of at least 400 feet per minute, reducing the cross-sectional area of the metal strip

- approximately 50 per cent on its first pass therethrough, and further reducing its cross-sectional area at least an additional 30 per cent on each succeeding pass.
5. A method of working a thin and relatively wide metal strip which includes moving the same through a single-stand cold-rolling mill at a linear speed of at least 400 feet per minute, reducing the cross-sectional area of the metal strip
- 10 10. approximately 50 per cent on its first pass, further reducing its cross-sectional area approximately 45 per cent in a succeeding pass through the mill, and finally reducing the cross-sectional area of the metal strip an approximate additional
- 15 15. 35 per cent, whereby the total reduction in the cross-sectional area of the metal strip in the single-stand cold-rolling mill is approximately 82 per cent while confined to only three passes therethrough.
- 20 20. 5. The method of working a thin and relatively wide metal strip which includes moving the same through a single-stand cold-rolling mill, reducing the cross-sectional area of the metal strip approximately 35 per cent on its first pass there-

through, and further reducing its cross-sectional area at least 35 per cent in a single succeeding pass while moving the strip at a speed of approximately 800 feet per minute.

6. A method of working a thin and relatively wide metal strip in a single-stand cold-rolling mill employing a pair of metal-working rolls of which at least one is slightly convex and a pair of substantially cylindrical backing-up rolls, which includes the steps of disposing the metal strip between the metal-working rolls, tightening the mill screws until the convexity of the slightly convex metal-working roll is taken up by the spring inherent in all of said rolls, whereby the mill provides a substantially flat active metal 10 pass under high screw pressure, moving the metal strip through said mill at a linear speed of at least 400 feet per minute, reducing the cross-sectional area of the metal strip at least 35 per cent on its first pass therethrough and further reducing its cross-sectional area at least an additional 35 per cent while confining the same to not more than three passes after the first pass.

HOWARD G. McILVRIED.